

Patented Feb. 20, 1923.

1,446,104

# UNITED STATES PATENT OFFICE.

JOHN H. RAVEN, OF CHICAGO, ILLINOIS.

## COATING FOR TRANSFER PAPER.

No Drawing.

Application filed August 12, 1922. Serial No. 581,544.

To all whom it may concern:

Be it known that I, JOHN H. RAVEN, a citizen of the United States, and a resident of the city of Chicago, in the county of Cook and State of Illinois, have invented a new and useful Coating for Transfer Paper; and I do hereby declare that the following is a full, clear, and exact description of the same.

In the making of lithographs the design upon a stone or plate in lithographic ink or color is handled by means of a paper coated with a suitable adhesive. This paper, which is known as transfer paper, is applied to the stone or plate so that the design is reproduced thereon. For commercial work it is very soft and tough paper such as India paper or rice paper, but for color work other paper may be used. After it has been applied to the stone so as to receive the design, it is removed and fastened to a sheet known as the layout sheet. The pattern upon the stone can thus be repeated a number of times upon the layout sheet, a separate sheet of transfer paper being used for every repetition of the pattern so that the layout comprises a foundation sheet of ordinary paper, having a number of pieces of transfer paper thereon, the coated side of the transfer paper being away from the foundation sheet and the paper being secured to the foundation sheet in any convenient way such as pricking with a needle.

The layout sheet with the transfer paper thereon is then put to one side until a convenient time for the printing. When this time arrives, the first step is to apply the layout sheet to the zinc, stone or other plate that is to be used for printing, the adhesive side of the transfer paper being next to the stone or plate. By the proper application of pressure the pattern is then made to appear upon the stone or zinc. Then pulling the transfer paper off leaves the protective ink on the stone or plate in the desired pattern, so that the plate may be etched in any of the usual ways.

In this process, the time during which the layout sheet may be put aside has heretofore been limited by the character of the coating upon the sheet, particularly in hot weather. If an attempt is made to keep the layout sheet too long before applying it to the stone or plate, it will fail to adhere and the pattern thereon will not be properly reproduced. The character of the adhesive used

has also limited the number of layout sheets that can be piled upon each other, because if too large a number are so piled they will stick to each other and the patterns on them will thus be lost.

It is an object of the present invention to produce a transfer paper so coated that the layout sheet may be kept much longer than heretofore, even in hot and damp weather.

It is a further object of this invention to produce a transfer paper with a coating that shall maintain its necessary adhesive qualities as long as the ink used thereon remains fresh enough to be transferable.

It is a further object of this invention to produce a coating for transfer paper which shall be made without the use of dextrine or glue, gelatine, or other product of animal nitrogenous matter.

It is a further object of this invention to produce a coating for transfer paper which shall be made wholly of starchy or farinaceous material except for the addition of an antiseptic, such as salt.

It is a further object of this invention to prepare a coating for transfer paper which shall be free from any tendency to become lumpy or granulated, and so will continue to produce a uniform smooth coating.

It is a further object of this invention to produce a transfer paper that shall require a considerable pressure to make it adhere to other sheets so that they may be piled higher than has heretofore been the practice.

It is a further object of this invention to prepare a material for coating transfer paper which will yield a coating that will maintain its adhesive qualities for a long period.

Other and further objects of this invention will be apparent from the disclosures in the following specification, which sets out a preferred form of the invention.

In the preparation of the material for coating transfer paper, I take two ounces of table salt, dissolve the same in a pint of water, and let the solution stand for at least twenty-four hours so that all of the salt is completely dissolved. I then make a mixture of nine ounces of starch (either corn, wheat, potato or other starch) and five ounces of wheat flour. To this I add the pint of salt solution, and stir the result into three quarts of boiling water. This makes

2  
a thick paste to which I add twelve ounces of pure glycerine. The batter is then stirred until thoroughly mixed and cool enough to handle in applying it to the paper. Preferably the batter is strained through a fine sieve while cooling.

The resulting mixture will be a batter of a consistency that will drip from a mixing spoon but will not quickly flow therefrom. 10 The batter is spread over the surface of the paper and smoothed by a coating machine or by the workman's forearm in the manner well understood by those skilled in this art. The paper is then ready to apply at 15 once to the stone or plate. If not at once thus applied, the paper will still be fit for use even if kept some weeks in warm weather. In cool weather it will keep indefinitely. It can be shipped in mailing tubes to be used by lithographers at distant 20 points.

If the transfer paper is applied to the stone or plate while still fresh, the layout sheets can be kept in piles of more sheets 25 than heretofore and even in warm weather the adhesive will continue in workable condition much longer than heretofore, and even longer than the ink of the design will.

It is of course understood that the 30 portion of water and glycerine must be varied to correspond to the weather, a smaller proportion of glycerine being used in damp weather. I am aware also that proportions of the other ingredients may be varied 35 through a wide range and that the details of the several steps of the process can be largely changed without departing from the spirit of this invention, and I therefore do not wish to limit the patent granted 40 hereon otherwise than is necessitated by the prior art.

I claim as my invention:

1. A coating for lithographic transfer paper comprising from one-third of an ounce 45 to one pound flour, one pound starch, from one-half to twenty ounces salt, from two to

fifteen quarts water, and from three to twenty fluid ounces glycerine.

2. A coating for lithographic transfer paper comprising a mixture of one pound 50 starchy material, one to two pints of a solution of common salt containing from one-fourth of an ounce to the pint to saturation, and from eight to thirty ounces of glycerine.

3. A coating for lithographic transfer paper, comprising a mixture of starchy material, a solution of common salt and glycerine in substantially the proportions specified, said mixture being free from non-starchy adhesives. 55

4. A process of coating paper to prepare a transfer paper which consists in dissolving common salt in water from one-fourth of an ounce to the pint to saturation, permitting the solution to stand until the salt 65 has completely dissolved, making a paste of flour, starch, from one-thirtieth to twice as much flour as starch, water, and the solution of salt, from one-half to four pounds of the dry material to a gallon of liquid, 70 adding glycerine to the resultant mixture in amount dependent on the weather, and applying the result to one surface of the paper.

5. A transfer paper coated with adhesive 75 material which will keep its adhesive properties for a period longer than it requires lithographic ink to dry.

6. A transfer paper comprising a sheet of paper coated on one side with an adhesive compound consisting of from one to twenty ounces flour, two pounds starch, sufficient water to form a thin paste, glycerine and two to fifteen ounces salt, without the admixture of animal adhesive substances. 85

In testimony whereof I have hereunto subscribed my name in the presence of two subscribing witnesses.

JOHN H. RAVEN.

Witnesses:

CARLTON HILL,  
OSCAR HARTMANN.